

J. H. YOUNG.  
PROTECTED METAL ARTICLE.  
APPLICATION FILED MAR. 26, 1921.

1,418,349.

Patented June 6, 1922.



Inventor:  
James Howard Young  
by Jas. H. Churchill,  
atty.

# UNITED STATES PATENT OFFICE.

JAMES HOWARD YOUNG, OF PITTSBURGH, PENNSYLVANIA, ASSIGNOR TO H. H. ROBERTSON COMPANY, OF PITTSBURGH, PENNSYLVANIA, A CORPORATION OF PENNSYLVANIA.

## PROTECTED METAL ARTICLE.

1,418,349.

Specification of Letters Patent. Patented June 6, 1922.

Application filed March 26, 1921. Serial No. 455,970.

To all whom it may concern:

Be it known that I, JAMES HOWARD YOUNG, a citizen of the United States, residing in Pittsburgh, in the county of Allegheny and State of Pennsylvania, have invented an Improvement in Protected Metal Articles, of which the following description, in connection with the accompanying drawings, is a specification, like characters on the drawings representing like parts.

This invention relates to a protected metal article of that character in which an article of corrodible metal, such as iron or steel, is protected against corrosion by a layer of asphalt or like bituminous material alone or in conjunction with layers of fibrous material, such as asbestos, wool, or other fibrous felts.

Protective metal articles of the character described are efficient against corrosion as long as the bituminous layer remains intact, but where the bituminous layer is exposed, it is subject to the deleterious action of light, heat, and atmospheric conditions; also to abrasion and other mechanical actions in handling, crating and shipping, and in some cases to injury by adhesion of one protected article to another.

The present invention has for its object to provide a protected metal article of the character described, which is provided with a protective covering of homogeneous, substantially non-fibrous, non-metallic layers, which are not soluble in water. A suitable covering of this character is a layer of vegetable parchment, which may be produced by the use of sulphuric acid or through the use of zinc chloride in a manner well-known.

The covering of vegetable parchment is applied to the bituminous or like hydrocarbonaceous material, while the latter is in a tacky condition and is adhesively affixed thereto, and forms an effective protection for the latter against extraneous influences and against the escape of the volatile constituents of the bituminous layer.

The covering of vegetable parchment is preferably waterproofed, which may be effected in several ways, one very effective way being to coat it with a film of cellulose nitrate or acetate.

The particular features of the invention will be pointed out in the claims at the end of this specification.

Fig. 1 is a plan of a protected metal article embodying this invention, and

Fig. 2, a section on an enlarged scale on the line 2-2, Fig. 1.

Referring to the drawing, *a* represents an article of corrodible metal, such as iron or steel, which may be rigid or flexible and of any form, and which is herein represented as a metal sheet.

The article *a* is provided with a protective layer *b* of asphalt or hydrocarbonaceous material of like character, which may be applied in any suitable manner as by passing the article *a* through a bath of melted asphalt. The asphalt or like layer *b* has applied to it while in a tacky condition a layer *c* of vegetable parchment, preferably waterproofed by a film *d* of cellulose nitrate or acetate. The layer *c* is homogeneous, substantially non-fibrous and is not soluble in water, but as it has the property of absorbing more or less water when subjected to a long continued wetting, it is preferred to provide the parchment layer *c* with the waterproofing film *d*.

The layer *c* forms an effective barrier against the escape of the volatile constituents of the asphalt layer *b* and also against the action of external influences, and on account of its low cost it reduces to a minimum the cost of the protected metal article. It also is a reflector of light and heat and can be painted in any color with ordinary paints.

### Claims:

1. As an improved article of manufacture, a protected metal article comprising an article of corrodible metal, a layer of bituminous or like hydrocarbonaceous material covering said corrodible metal, and a layer of vegetable parchment adhesively affixed to said hydrocarbonaceous material.

2. As an improved article of manufacture, a protected metal article comprising an article of corrodible metal, a layer of bituminous or like hydrocarbonaceous material covering said corrodible metal, and a layer of waterproofed vegetable parchment ad-

hesively affixed to said hydrocarbonaceous material.

3. As an improved article of manufacture, a protected metal article comprising an article of corrodible metal, a layer of bituminous or like hydrocarbonaceous material covering said corrodible metal, and a layer

of vegetable parchment adhesively affixed to said hydrocarbonaceous material and provided with a waterproofing film of cellulose derivative.

In testimony whereof, I have signed my name to this specification.

JAMES HOWARD YOUNG.